

## UNITED STATES PATENT OFFICE

1,946,670

FERRO-TITANIUM ALLOY AND METHOD OF  
MAKING SAME

George F. Comstock, Niagara Falls, N. Y., assignor to The Titanium Alloy Manufacturing Company, New York, N. Y., a corporation of Maine

No Drawing. Application August 14, 1931  
Serial No. 557,135

5 Claims. (Cl. 75—22.5)

My invention relates generally to titanium alloys for the treatment of ferro-metals and more particularly to the methods of making such an alloy for treating iron and steel to remove therefrom gaseous or other impurities that have injurious effects upon the metal and to modify the properties of such metals by incorporating therewith titanium and silicon.

The ferro-titanium alloys now in common use are made either with about 7% carbon to insure freedom from the comparatively inactive nitride, or by the aluminothermic process to give a low-carbon alloy of low melting point. Other ferro-titanium alloys containing silicon have been described, but are not widely used, probably because of too high a melting point. The fusion temperature of these alloys varies directly with the carbon content, so that for low melting points a low carbon content is essential.

For general use as a deoxidizer and scavenger of molten steel, the ferro-carbon-titanium containing about 7% carbon has a wide field of usefulness, and is the least expensive form of titanium available, on account of ease of manufacture. For certain purposes however a low carbon alloy is desirable, as for example, when a content of metallic titanium, as distinct from titanium-carbide, is desired in an alloy steel, or when the titanium alloy used must have a low fusion temperature as in treating small quantities of steel or cast iron where rapid absorption of the alloy in the melt is essential.

The only alloys heretofore available for such purposes are the aluminothermic ferro-titanium, which suffers from the objection of an aluminum content, not desired in many steels which must be as clean as possible; and certain alloys containing titanium and silicon. The latter, as described in the literature, have been made in such a way as would inevitably result in a carbon content greatly above 1%, so that the fusion point would be not low enough to compensate for the additional cost of such alloys as compared with the more generally used and well known ferro-carbon-titanium.

I have discovered a new ferro-titanium alloy containing silicon, which has a low melting point and can be made without difficulty in an ordinary electric furnace. The alloy contains not over 1% carbon, and it is also practically free from aluminum, thus permitting it to be used in steels where no inclusions of alumina are permissible. It can be used to confer the benefits of titanium-treatment on gray cast iron in small ladles, and the strength of the iron is increased

about 25% by such treatment. Thus high-strength iron may be made in small amounts when desired from a cupola-run of ordinary iron without changing the charge in the cupola. When incorporated in the flux coating on electric welding rods in a finely-divided form, this improved alloy has been found to prevent the formation of oxide and nitride of iron in the deposited metal, which is thus made similar in structure to a steel casting.

My improved titanium alloy is readily made in the usual carbon-lined furnace by the simultaneous reduction of ilmenite which is a ferrous-titanate ( $FeTiO_3$ ) containing about 55% titanium oxide with the balance iron oxide and silica rock or quartz containing about 98% silica. These ingredients are preferably crushed to about half-inch size, though any size available between 40-mesh and one inch lumps may be used.

"Barley" coal is used for reduction, and a small amount of ferro-carbon-titanium, for example that described in the U. S. Rossi and Meredith Patent No. 1,039,672 of September 24, 1912, crushed to about  $\frac{1}{8}$  to  $\frac{1}{4}$  inch size, is added in place of the usual scrap iron in order to increase the electrical conductivity of the charge. This substitution of the high-carbon titanium alloy for scrap-iron in the charge is an essential part of my improved methods, for by this means I have found it possible to obtain a satisfactory content of titanium in the product without raising the carbon content too high for good fusibility. If scrap-iron is used in the charge, and the titanium content of the product is raised by increasing the proportion of titanium ore to silica in the charge, it is found that the carbon content rises with it, something I wish to avoid as hereinbefore described. But by using ferro-carbon-titanium in the charge in place of scrap-iron, it is possible to so adjust the proportions of titanium ore and silica used as to obtain a new low carbon ferro-titanium alloy containing over 15% titanium with silicon content about 20% and not over 1% carbon.

Such alloy made in this way contains 15 to 25% each of titanium and silicon, and less than 1% each of carbon and aluminum, the balance, or about 55 to 60%, being iron. An example of a furnace charge which has been used successfully is as follows:— 32% ilmenite, 38% silica, 15% ferro-carbon-titanium, and 15% coal. Variations of this charge within approximately the following limits are probably permissible:— Ilmenite 30 to 35%; silica 35 to 40%; ferro-car-

bon-titanium 12 to 18%; coal 12 to 20%. The coal may be so distributed through the mix to be charged that more is added in the final portions of the furnace charge than in the portions that are in the furnace longer. The furnace should be charged slowly, and should be tapped 20 to 30 minutes after the last of the charge is melted, as by that time most of the melt should have been reduced to metal.

10 I claim as my invention:

1. A low-carbon, silicon-containing, ferro-titanium alloy having a low melting point and being practically free from aluminum, and embodying a titanium content from 15 to 25%, a silicon content about 20%, from a trace to less than 1% of carbon, and the balance substantially iron.

2. A low-carbon, silicon-containing, ferro-titanium alloy having a low melting point and being practically free from aluminum, and embodying a titanium content from 15 to 25%, a silicon content about 20%, about 0.5% of carbon, and the balance substantially iron.

20 3. In the method of making a low-melting, silicon-containing, ferro-titanium alloy, practically free from aluminum, the step which consists in reducing titaniferous ore and silica in a

carbon-lined furnace in the presence of ferro-carbon-titanium, the charge containing a reducing agent and a preponderating amount of iron for the production of said ferro-alloy having a titanium content above 15%, a silicon content less than 25%, and carbon less than 1%.

5 4. In the method of making a low-melting ferro-titanium alloy the step which consists in reducing in a carbon-lined electric furnace a charge containing approximately the following ingredients: ilmenite (30 to 35%); silica (35 to 40%); ferro-carbon-titanium (12 to 18%); and coal (12 to 20%) to form a ferro-titanium alloy containing over 15% titanium with silicon content about 20% and not over 1% of carbon.

10 5. In the method of making a low-melting, silicon-containing, ferro-titanium alloy, practically free from aluminum, the step which consists in reducing in a carbon-lined electric furnace a charge containing approximately the following ingredients: ilmenite 32%; silica 38%; ferro-carbon-titanium 15%; and coal 15%, to form a ferro-titanium alloy containing over 15% titanium with the silicon content about 20% and not over 1% of carbon.

90 100  
GEORGE F. COMSTOCK.

105  
50

110  
35

115  
40

120  
45

125  
50

130  
55

135  
60

140  
65

145  
70

150  
75